

## UNITED STATES PATENT OFFICE

2,311,931

## LUBRICANT

Elmer William Cook, New York, N. Y., and William David Thomas, Jr., Stamford, Conn., assignors to American Cyanamid Company, New York, N. Y., a corporation of Maine

No Drawing. Application December 27, 1941,  
Serial No. 424,600

5 Claims. (CL 252—48)

This invention relates to lubricants of improved characteristics containing new organic compounds which possess detergent, anti-corrosion, film-forming and other valuable properties when dispersed therein.

The new compounds of our invention to be described herein may be designated as metal salts of alkyl or cycloalkyl salicylate sulfides having the general formula



in which  $R_1$  and  $R_2$  are alkyl or cycloalkyl radicals having 4 or more carbon atoms,  $n$  is a positive integer not more than 2,  $M$  is a metal radical and  $X$  is the valence of  $M$ .

These compounds are particularly valuable as additives to lubricating oils used in heavy duty service and under extreme pressure conditions because of the unique detergent, anti-corrosion, film-forming and other properties which they possess. When conventional hydrocarbon lubricating oils are subjected to high operating temperatures for long periods of time, as in heavy duty service, they tend to decompose with the formation of complex oxidation and decomposition products. These acidic oxidation products corrode certain alloy bearings such as copper-lead, silver-cadmium, nickel-cadmium, etc. which are commonly employed in internal combustion engines. These decomposition products also tend to polymerize under the high temperature conditions obtaining in the engine to form sludge which precipitates when the engine is cooled or when fresh oil is added. The precipitated sludge clogs the oil filter and becomes caked on heated metal surfaces to form lacquer-like deposits which may cause the piston rings or even the piston itself to stick.

Attempts have been made to overcome these deficiencies of the lubricating oil by the addition of detergents or anti-corrosion agents, or both. Certain anti-corrosion agents, such as triphenyl phosphite and sulfurized sperm oil, counteract the corrosive effect of the oxidation products formed in the oil. These anti-corrosion agents have no detergent properties, however, and while they cover the bearing surfaces and other corrodable parts of the engine with a passivating film that prevents corrosion of the metal by the organic acids of the oil, they do not act to dis-

perse the sludge or prevent the formation of the varnish deposits mentioned above.

A number of oil-soluble detergents of the type of metal soaps, phenolates and alcoholates have been proposed and used in crankcase oils to dissolve or disperse the sludge and prevent varnish deposits and piston ring sticking. Unfortunately, however, the greater majority of these substances increase the rate of oxidation in a manner somewhat analogous to the accelerating action of the various metallic soaps or "driers" on the oxidation of varnish films, and their presence results in an increased concentration of acidic oxidation products in the oil. When individual detergents and anticorrosion agents are used together in the oil the two separate chemicals do not cooperate to reduce corrosion and sludge and varnish formation. The lack of cooperative effect is believed to be due to the action of the detergent in removing from the metal surfaces the passivating film of anti-corrosion agent which is supposed to cover the metal surface and thereby prevent corrosion.

The compounds of the present invention show both excellent detergent and excellent anti-corrosive action when dispersed in lubricating oils and thereby enable us to provide a lubricating oil having a single additive effective to inhibit corrosion, sludge and varnish formation, ring sticking and other difficulties experienced in lubricating oils serving in a heavy-duty capacity. The addition of our compounds to lubricating oils also imparts to the oil a high film strength thus enabling the oil to be used under extreme pressure conditions under which the film formed by conventional oils would break and result in seizing of the bearing surfaces.

The extremely high solubility of these compounds in hydrocarbon oils leads to another important advantage, namely, the ease with which they are blended with lubricating oils. This step is further simplified by our practice of dissolving them in ordinary types of lubricating oils to the extent of 50% or more for storage and shipping purposes. For this reason it will be understood that the appended claims are intended to cover lubricating compositions containing such high concentrations of our new compounds.

Another advantage to be obtained by the use of our alkyl and cyclo-alkyl salicylate sulfides is their solubilizing action on certain materials which are known to be good detergents, anti-oxidants, etc. or have good corrosion inhibiting properties but which cannot normally be used in

high concentrations on account of their oil insolubility. Certain dithiophosphates, such as di(para-tertiary amyl phenyl) dithiophosphate; calcium, barium, aluminum, zinc, and magnesium stearates, palmitates, naphthenates; etc. are difficultly soluble in lubricating oils, but because of their solubility in the compounds described herein, it is possible to add them to oils in this way in amounts sufficiently large for them to be effective.

The compounds of the present invention may be prepared by reacting an aliphatic or cyclo-aliphatic ester of salicylic acid with sulfur chloride ( $S_2Cl_2$ ), sulfur di-chloride ( $SCl_2$ ), or thionyl chloride ( $SOCl_2$ ) in the presence of Cu, depending upon whether a mono-sulfide or di-sulfide is desired as the reaction product. We prefer the mono-sulfides because of their greater chemical stability. The monosulfides are prepared by reacting approximately 2 mols of an aliphatic or cyclo-aliphatic ester of salicylic acid with 1 mol of sulfur dichloride in the presence of a small amount, for example 0.2 mol, of anhydrous  $AlCl_3$  as catalyst. Other Friedel-Crafts catalysts, such as  $SbCl_3$ ,  $FeCl_3$ ,  $TeCl_4$ ,  $SnCl_4$ ,  $TiCl_4$ ,  $TeCl_4$ ,  $BiCl_3$  and  $ZnCl_2$  may also be employed as catalysts in our reaction, but with decreasingly effective results. The disulfides are prepared in the same manner by substituting sulfur chloride in place of sulfur dichloride. The reaction may be illustrated as follows:



The product illustrated is then treated with a metal oxide or hydroxide to prepare salts having the general formula:



in which  $R_1$ ,  $R_2$ ,  $M$  and  $X$  are as indicated in the general formula described above.

The metal radicals which we introduce into our alkyl or cycloalkyl salicylate sulfides to form salts thereof, include metal radicals such as aluminum, lead, magnesium, zinc, calcium, barium, strontium, sodium, potassium, etc. The metal salts of our invention may be prepared by simply neutralizing the alkyl or cycloalkyl salicylate sulfides with an appropriate metal oxide or hydroxide or, if desired, by methods of double decomposition. For purposes of improving lubricants we prefer to employ the alkaline earth metal salts since they possess greater detergency and heat stability.

The salicylic acid ester employed in the above reaction should be an ester of an aliphatic or cyclo-aliphatic alcohol having at least 4 carbon atoms so that  $R_1$  and  $R_2$  in the general formula may be alkyl or cycloalkyl radicals of at least 4 carbon atoms. The size of the alkyl or cycloalkyl radical is important in that the higher molecular weight radicals promote the solubility of our compounds in lubricating oils and the radicals should be of at least the size indicated in order that our compounds may be dissolved in

the lubricant without undue difficulty.  $R_1$  and  $R_2$  may therefore be alkyl radicals such as butyl, normal amyl, tertiary amyl, ethyl hexyl, normal octyl, decyl, dodecyl, hexadecyl, octadecyl, etc. or cyclo-aliphatic radicals such as cyclopentyl; cyclo hexyl, methyl, ethyl, propyl, butyl, and amyl, mono-, di-, and tri-substituted cyclo hexyl radicals, etc.

Ordinarily we carry out the reaction with the reactants dissolved in a suitable solvent such as carbon disulfide, ethylene chloride, petroleum naphtha, nitrobenzene, etc. The reaction mixture with a catalyst present is then heated until the evolution of  $HCl$  has substantially stopped. The mixture is then treated with cool dilute hydrochloric acid or other acids such as sulphuric, acetic, etc. and the product recovered by extraction with toluene or other solvents. The product can be further purified by washing with water in which it is insoluble and the solvents removed by evaporation.

It will be understood, of course, that the preparation of the disulfide with sulphur chloride proceeds in the same way under the same reaction conditions. It will also be understood that the cyclo-aliphatic esters of salicylic acid may be employed in place of the aliphatic esters of salicylic acid illustrated in the above illustration in the same manner and using the same molecular proportions.

The preparation of barium dodecyl salicylate monosulfide will now be described in detail in the following example in which particular parts of the reactants, catalysts, solvents, etc. are indicated merely for purposes of illustration. It will also be understood that our invention is not to be limited to the particular compound described since as stated above the invention is of broader scope and is to be limited only by the scope of the appended claims. The parts indicated are by weight.

#### Example

150 parts by weight of dodecyl (lauryl) salicylate was condensed with 24 parts of sulfur dichloride in 30 parts of A. S. T. M. naphtha in the presence of 8 parts of  $AlCl_3$  as catalyst. Condensation was carried out by warming the reaction mixture on a steam bath between 60-70° C. with stirring for 30 minutes. The reaction mixture was then cooled and diluted with cold dilute hydrochloric acid, extracted with toluene, washed and the solvent evaporated. Dodecyl salicylate monosulfide was removed as a brownish-yellow liquid.

The barium salt of dodecyl salicylate monosulfide was prepared by neutralizing 40 parts of dodecyl salicylate monosulfide with 18 parts of barium hydrate in a solution of 20 parts of ethyl alcohol and 16 parts of toluene with stirring at 70° C. As the solvent evaporated fresh toluene was added from time to time and the heating increased to a temperature of 110° C. The solution was then filtered from traces of inorganic salts and then evaporated, the last of the solvent being evaporated under reduced pressure. 55 parts of barium dodecyl salicylate monosulfide was obtained which was dissolved in an equal amount of lubricating oil for storage and blending purposes.

The compounds as described above are heat stable and not easily decomposed in the lubricant because of high operating temperatures which may be encountered. They are also practically water-insoluble and are not extracted from the

lubricant by contact with water nor do they appreciably promote the formation of emulsions with water in the oil.

The metal salts of alkyl and cyclo-alkyl salicylate sulfides are so very effective as detergents and as corrosion inhibitors that it is possible to improve lubricating oils, particularly those of the crankcase type, to a great extent by the use of very small amounts of the compound. In lubricating oils intended for ordinary purposes where high temperatures occur only occasionally, from 0.1 to 0.8% of the metal salt of the alkyl or cycloalkyl salicylate monosulfide is sufficient. In extreme pressure lubricants and in oils intended for heavy duty service, it is generally advisable to use a little more, as for example 0.5 to 3.0% of the oil.

The effectiveness of our compounds in lubricating oils as corrosion inhibitors, detergents and anti-oxidants was demonstrated by the results obtained upon subjecting a No. 30-W grade Mid-Continent solvent refined oil to the Catalytic Indiana Test. This test was conducted in an apparatus consisting of a number of large glass test tubes immersed in a constant temperature bath maintained at 341° F. 300 cc. samples of the oil containing dispersed therein 0.4% of barium dodecyl salicylate monosulfide were poured into the tubes and air passed through the oil at the rate of 10 liters per hour. In order to simulate the conditions prevailing in the crankcase of an engine, weighed strips of copper-lead alloy were suspended in the oil. A test tube containing a sample of the same oil without benefit of the barium dodecyl salicylate monosulfide additive was used as a control. After subjecting the oil to the test for 70 hours, the copper-lead alloy strips were removed, washed and weighed. The copper-lead strips immersed in the lubricating oil containing no additive, showed a bearing loss of 275 mg. per sq. inch. The copper-lead strips immersed in the lubricating oil containing 0.4% of barium lauryl salicylate monosulfide showed, at the end of the 70 hour test, no corrosion loss whatever. After pouring out the oil and rinsing once with kerosene, the two test tubes

which had contained the oil with the barium dodecyl salicylate monosulfide additive was very clean, thus indicating that the oil with the additive had a high degree of detergency. The tube containing the oil without additive was very dirty. This test indicated clearly the remarkable corrosion inhibiting and detergent effects of our compounds in lubricating oils.

What we claim is:

1. A lubricating composition comprising a major proportion of a lubricant having dispersed therein a minor proportion of a compound having the general formula



in which  $\text{R}_1$  and  $\text{R}_2$  are members of the group consisting of alkyl and cycloalkyl radicals having 4 or more carbon atoms,  $n$  is a positive integer and not more than 2,  $M$  is a metal radical and  $X$  is the valence of  $M$ .

2. A lubricating composition comprising a major proportion of a lubricant having dispersed therein a minor proportion of a compound having the general formula



in which  $\text{R}_1$  and  $\text{R}_2$  are members of the group consisting of alkyl and cycloalkyl radicals having 4 or more carbon atoms, and  $M$  is an alkaline earth metal radical.

3. A lubricating oil having dispersed therein 0.1-3% of barium dodecyl salicylate monosulfide.  
 4. A lubricating oil having dispersed therein 0.1-3% of barium octyl salicylate monosulfide.  
 5. A lubricating oil having dispersed therein 0.1-3% of barium decyl salicylate monosulfide.

ELMER WILLIAM COOK.  
 WILLIAM DAVID THOMAS, JR.